

# UNITED STATES PATENT OFFICE.

GUY D. HARPER, OF FRANKLIN, PENNSYLVANIA.

## METHOD OF PRODUCING LUBRICATING OILS.

1,414,695.

Specification of Letters Patent. Patented May 2, 1922.

No Drawing.

Application filed May 11, 1918. Serial No. 233,849.

To all whom it may concern:

Be it known that I, GUY D. HARPER, citizen of the United States, residing at Franklin, in the county of Venango and State of Pennsylvania, have invented certain new and useful Improvements in Methods of Producing Lubricating Oil, of which the following is a specification.

This invention relates to improvements in the art of producing lubricating oil from crude petroleum by the combined operations of concentration and filtration.

More especially, this invention relates to the art of converting a crude petroleum having a so-called naphthene base into a lubricating oil that is particularly suitable, on account of its low carbon content, for lubricating internal combustion motors.

The crude petroleum for which my process has been found most suitable, has, as previously stated, a so-called naphthene base, and the following characteristics at the time it is pumped from the well, or shortly thereafter:

|                      |               |
|----------------------|---------------|
| 25 Gravity at 60° F. | 29 to 31 B.   |
| Flash test           | 130 to 165 F. |
| Fire test            | 160 to 230 F. |
| Cold test            | — 25 F.       |

30 The lubricating oil which I produce by said process has the following characteristics:

|                      |                           |
|----------------------|---------------------------|
| Gravity at 60° F.    | 28 to 30 B.               |
| Flash                | 400° to 450° F.           |
| Fire                 | 465° F.                   |
| Viscosity at 100° F. | 468, (Saybolt universal). |
| Cold test            | 30° to 40 F.              |
| Carbon content       | 69/100 of one per cent.   |

40 The process which I employ in the production of said lubricating oil is substantially as follows:

When the crude petroleum is pumped from the wells, it is placed in open tanks, and the water which is mingled with it is permitted to settle to the bottom of the tank; the foreign matter, such as silt, etc., settles out to some extent at the same time. The length of time allowed for this settling operation is variable, and depends somewhat upon the temperature, but ten days may generally be considered sufficient.

45 After being so treated, the crude oil is passed through a filter containing a suitable

filtering medium, such as bone-black or fullers' earth, and after being thus filtered the oil is placed in a still and gradually heated, first, preferably by means of heat applied externally to the still; the condenser 60 pipe leading from the still is allowed to remain open during the whole time of the application of heat: When the temperature of the stock within the still reaches the point of 190° F. or very close to that point, vaporization begins to take place.

When the temperature of said stock has reached said point of 190° F., more or less, through the application of external heat, steam is admitted to the still, and delivered 70 thereinto at a point close to the bottom of said still, beneath the body of stock, preferably through a pipe having small perforations extending the full length of the still, so that the heat is evenly applied. Through 75 the medium of such applied steam the temperature of the stock is very gradually brought to the point of 370° F., more or less, the steam being heated to impart such temperature thereto.

When said last mentioned temperature has been imparted to the stock the application of heat is gradually diminished and finally entirely discontinued. This leaves the stock in a highly heated condition and vaporization will continue for sometime until the temperature falls below the vaporization point. The oil remaining in the still after vaporization ceases will be found to be approximately 70% original stock, approximately 30% having been driven off in the form of vapor distillate. The tail-pipe to the condenser remains open throughout the operation, thus permitting the escape of all vapor, in order that the concentration, or 85 distillation, as above mentioned, may continue so long as there is sufficient heat to produce a vapor, or until the residue has been removed from the still.

After the concentrated oil has become cool 100 it is passed through a filter containing a suitable filtering medium, such as bone-black or fullers' earth. It may be passed through the filter several times if desired, to lighten the color.

105 In specifying the above amount of distillate as 30% of the original stock, and the residual product as 70%, it should be understood that these quantities may vary either way to a considerable extent, as, for illustra- 110

tion, when the crude is fresh from the well, the distil ate will be in excess of said 30% and the residual product, or concentrated oil a less quantity than 70%. Likewise, if the 5 crude stock has remained for a considerable period of time in the open tanks, said variation will be in the opposite direction, and the heat applied to the still should be regulated with proper consideration for these 10 conditions.

This process when applied to a crude oil having a naphthene base, produces a lubricating oil having the characteristics previously set forth, and, inasmuch as no refining agents, such as soda, acid, etc., now 15 so commonly employed in oil refining operations, are used, my resulting lubricating oil is wholly free from injurious ingredients, has a high viscosity, and is markedly free 20 from carbon, which has been found to be troublesome in cylinders of internal combustion motors.

So far as known at present, however, the amount of petroleum produced in the United 25 States having a so-called naphthene base, does not equal two per cent of the whole quantity of petroleum produced, and there are only two or three small areas in the United States where such petroleum is 30 found.

Crude petroleum having the qualities and characteristics herein set forth, and for the refining of which the process herein set forth is suitable, is generally known as "Franklin 35 heavy oil" also as "first sand oil," and is produced at and in the vicinity of Franklin, Pennsylvania. This should not be understood as meaning what is generally known as Pennsylvania crude, as this latter crude has 40 a paraffine base, and requires a different process to convert it into a lubricating oil. While I have stated that the stock in the still is first brought to a temperature of 190° F. by means of fire heat, I do not wish to be 45 understood as being strictly confined to this restriction: The temperature of 190° F. is, however satisfactory, and a safe temperature to employ, but by careful and even firing and close attention, the temperature 50 of the stock may be brought, by fire heat to a point as high as 350° F. before steam is applied. It should be understood, and will be understood by those skilled in the art of refining petroleum, to produce lubricating 55 oil, that all of the various temperatures given, except those relating to gravity and viscosity, cannot always be attained and maintained with certainty, in the refining of petroleum on a commercial scale, where 60 three bodies of fluid are being dealt with, and it is not absolutely essential that they should be. Said temperatures are set forth as a 65 part in and reliable guide to the refiner, and will produce the desired results, but a variation of twenty-five per cent either way, un-

der certain conditions, be as near as they can be attained, and still good results will follow.

I claim the following:

1. The method of producing a lubricating 70 oil ready for commercial use as such which consists in selecting a crude petroleum of the grade of Franklin heavy oil and having a so-called naphthene base, concentrating the same by distillation to approximately 70% 75 of its original volume and then filtering the residual product to produce such lubricating oil.

2. The method of producing a lubricating 80 oil ready for commercial use as such which consists in selecting a crude petroleum of the grade of Franklin heavy oil and having a so-called naphthene base, driving off the lighter fractions therefrom by means of applied heat at a temperature of approximately 85 370° F., and then filtering the residual product to produce such lubricating oil.

3. The method of producing lubricating 90 oil ready for commercial use as such which consists in selecting a crude petroleum of the grade of Franklin heavy oil and having a so-called naphthene base, passing said petroleum through a suitable filtering medium, then extracting the distillate therefrom equal to 30% of the original volume by 95 means of applied heat, and then filtering the residual product to produce such lubricating oil.

4. The method of producing lubricating 100 oil ready for commercial use as such which consists in selecting a crude petroleum of the grade of Franklin heavy oil and having a so-called naphthene base, subjecting the same when pumped from the wells to the action of the atmosphere until the water 105 contained therein has settled, then passing the same through a filtering medium, then placing the same in a still and gradually applying heat thereto until the same has reached an approximate temperature of 110 370° F. during the time of applying such heat permitting the resultant vapor to escape from the still to approximately 30% of the original volume of stock, then cooling the residual product and then passing said 115 residual product through a suitable filtering medium to produce such lubricating oil.

5. The method of producing lubricating 120 oil ready for commercial use as such which consists in selecting crude petroleum of the grade of Franklin heavy oil and having a so-called naphthene base, separating the water therefrom by settling while exposed to the action of the atmosphere, then passing the oil through a suitable filtering medium, then placing the same in a still and subjecting it to heat gradually applied externally to the still until the stock has reached a temperature of approximately 125 190° F. and then gradually injecting steam 130

into and adjacent to the body of the stock and continuing such injection of steam until a temperature of approximately 370° F. is reached, and simultaneously with such application of heat permitting the resulting vapor to escape from the still to the extent of approximately 30% of the original volume of crude stock, then permitting the residual product to cool, and then passing 10 said residual product through a suitable filtering medium to produce such lubricating oil.

6. The method of producing a lubricating oil ready for commercial use as such which 15 consists in selecting crude petroleum of the grade of Franklin heavy oil and having a so-called naphthene base, a gravity of 29 to 31 B. at 60° F., a flash test of 130° to 165° F., a fire test of 160° to 230° F. and a cold 20 test of approximately -25° F., extracting the lighter fractions therefrom by distillation through the medium of applied heat whose maximum temperature is approximately 370° F. until approximately 70% of the 25 original stock remains, cooling the residual stock after such extraction and then filtering the same to produce such lubricating oil.

7. The method of producing a lubricating

oil ready for commercial use as such which consists in selecting crude petroleum of the 30 grade of Franklin heavy oil and having a so-called naphthene base, subjecting the same to the action of the atmosphere, then filtering the same, then extracting the lighter fractions therefrom to the amount of 30% of 35 the original crude stock by process of distillation, and then cooling and filtering the residue to produce such lubricating oil.

8. The method of producing lubricating oil ready for commercial use as such which 40 consists in selecting crude petroleum of the grade of Franklin heavy oil and having a so-called naphthene base, subjecting the same to the action of the atmosphere by exposing the same in open containers, then extracting the lighter fractions therefrom in quantity equaling approximately 30% of 45 the original crude stock by process of distillation, and then filtering the residue, whereby a lubricating oil is produced having the 50 following characteristics: gravity at 60° F., 29 to 31 B., flash 450° F., fire 465° F., viscosity at 100° F. 370 (Saybolt universal), and cold test 20° to 45° F.

In testimony whereof I affix my signature.  
GUY D. HARPER.